

Dec. 9, 1952

R. H. PREW

2,621,104

MATERIAL FOR PROTECTING METALS FROM TARNISH

Filed July 26, 1949

*Fig. 1.*



*Fig. 2*



Inventor:  
Robert H. Prew,  
by Emery, Booth, Townsend, Atlys  
Miller & Weidner

## UNITED STATES PATENT OFFICE

2,621,104

MATERIAL FOR PROTECTING METALS  
FROM TARNISHRobert H. Prew, Nashua, N. H., assignor to Nashua  
Corporation, Nashua, N. H., a corporation of  
Massachusetts

Application July 26, 1949, Serial No. 106,855

4 Claims. (Cl. 21—2.5)

1

This invention relates to a material which may constitute a wrapper, a container wall, a lining for such a wall, or a wrapper to receive metal articles, notably those in whole or in part of silver, which are subject to tarnish from tarnishing agents in the atmosphere, notably sulphur or gases containing sulphur.

The formation on silver of the tarnish of silver sulphide is well known. It has been proposed to protect the silver by wrapping or packaging it in a textile fabric impregnated with some agent which because of its chemical nature or its physical form, or both, will be more susceptible to attack by sulphur than the silver piece itself. A somewhat extended discussion of this subject matter will be found in the patent to Jones 1,766,646. No novel chemical action is involved in the present invention and insofar as the choice of chemical agents is concerned it may be practiced by utilizing the knowledge of the prior art as for example said patent to Jones.

While the fabric impregnated with finely divided silver oxide as described in the Jones patent is, both in theory and practice, efficient in minimizing the tarnishing of silver, it has the disadvantage that when it operates by reaction of the silver salt with tarnishing gases such as hydrogen sulphide, the fabric becomes dirty and unattractive. In practice the invention has been utilized only with dark colors, minimizing this effect. Even among dark colors dull shades only may be used. A bright shade of a dark color could not be used.

The present invention provides a construction having an attractive texture capable of being produced in a wide variety of colors and which, while efficient in its anti-tarnishing action, does not noticeably deteriorate in appearance.

The material embodying the invention may be used for protecting articles subject to deleterious tarnishing, such as silver tableware, (flatware so-called), hollowware for use or ornament, ornamental articles including jewelry, in all instances whether sterling silver or silver plated or having a surface partly of silver, and also silver-gilt and rhodium plate on brass or slush metal, so-called, which latter is an alloy of zinc, lead and antimony. For convenience herein I designate all such articles by the term silverware.

The invention will be well understood by reference to the following description taken in connection with the accompanying drawing wherein:

Fig. 1 is a schematic and unrealistic view showing the improved material in section; and

Fig. 2 is a diagrammatic view illustrating a 55 in the fibers of the flock in finely divided form,

2

method of manufacturing the same, when a flexible backing is utilized.

The material of my invention in appearance has a surface resembling that of velvet and, when 5 incorporating a flexible backing as herein specifically described, is as a whole like a piece of velvet. Referring to Fig. 1 it may comprise a backing sheet 10 which may be a textile fabric, paper, or some other flexible sheeting having one face completely covered by a pile of upstanding filaments 12 and 14 of textile fiber which are secured thereto by suitable adhesive 16. This pile surface comprises long filaments 12 and short filaments 14 in substantially uniform relative distribution 10 throughout the area of the fabric. The long filaments 12 are sufficiently numerous to constitute the visible face of the right side of the fabric as in the case of the pile on a piece of velvet. While the short filaments constitute a substantial 15 proportion of the whole, the long filaments project beyond them as seen in Fig. 1 and substantially hide them. The construction may be compared to that of the pelts of certain fur-bearing animals, in which there is a fine inner fur which 20 is covered by longer, exposed hair.

In accordance with the invention the short pile 25 elements 14 carry a suitable anti-tarnish agent of any desired character as, for example, finely divided silver oxide precipitated in the fibers thereof, as described in the Jones patent aforementioned. Silver oxide is believed to be most efficient and is recommended. The long filaments are substantially free from such material.

The long filaments 12 determine the exterior 30 appearance of the material as a whole, which as already stated is that of velvet, and they may be of a bright color. Tarnishing gases readily penetrate the pile to react with the silver oxide on the short filaments. The resultant discoloration 35 however is dissimulated by the untreated long fibers 12, which hide the discolored short filaments.

In Fig. 2 I have shown diagrammatically one 40 manner in which the improved material may be produced on a backing 18 of textile fabric, paper, or other sheet material. A suitable material for use in forming the filaments is cut rayon flock. The short filaments 14 may be about one millimeter in length on the average and the long 45 filaments about two millimeters. As illustrated diagrammatically at the right of Fig. 2, the short filaments may be impregnated with silver nitrate solution and then treated with hot sodium carbonate solution, thus precipitating silver oxide 50 in the fibers of the flock in finely divided form,

which physical form is an important feature in their preferential susceptibility to the action of sulphur as contrasted with the solid metal of the articles which they are to protect. The flocks are then washed and dried as indicated by the legend of the drawing. Conveniently the treated short filaments and the untreated long filaments may be mixed and delivered to the distributing hopper 18 of a suitable flocking machine such as is shown diagrammatically in the lower portion of Fig. 2. The backing 10 is drawn from the roll at the right and a roller 20 spreads the adhesive 16 on its face. The adhesive side passes under the hopper 18 and the flock is shaken thereon, after which the sheet is subjected to the action of beaters 22 causing the flock elements to stand on end so that the lower ends are anchored in the adhesive 16 as shown in Fig. 1, from which they project substantially uniformly as long pile with a shorter pile received inwardly of the outer surface of the longer pile. Surplus flock is drawn away by an exhausting mechanism at 24 and the coated material passes through a drier 26 to set the adhesive and the completed sheet may then be rewound.

The material, depending somewhat on the nature of the backing 10, may be used as a container, as a wrapper, as a bag or as a lining for a box, cabinet or drawer for protecting silverware when in the hands of the ultimate consumer or at any or all stages of its transit from the manufacturer to the consumer.

I am aware that the invention may be embodied in other specific forms without departing from the spirit or essential attributes thereof, and I therefore desire the present embodiment to be considered in all respects as illustrative and not restrictive, as is in fact clear in several matters from the description itself. Reference is to be had to the appended claims to indicate those principles of the invention exemplified by the particular embodiment described and which I desire to secure by Letters Patent.

I claim:

1. Material for protecting from tarnish silverware placed in adjacency thereto, comprising a backing one face of which is covered by a pile consisting of relatively long and relatively short textile flock in substantially uniform relative distribution throughout the area of the backing, the flocks being adhesively secured endwise to the face of the backing in upstanding position, the short flocks retaining in the fibers thereof a sub-

stance which as compared with the silverware is preferentially susceptible to chemical attack by tarnishing agents in the air, the long flocks being substantially free of such substance.

2. Material for protecting from tarnish silverware placed in adjacency thereto, comprising a backing having relatively short and relatively long filaments secured thereto in the manner of a pile, the short filaments carrying silver in a form which will preferentially combine with the tarnishing agents in the atmosphere and prevent them from combining with the silver on the surface of the silverware and the long filaments being substantially free of such substance and projecting beyond the short and substantially hiding the same.

3. Material for protecting from tarnish silverware placed in adjacency thereto, comprising a backing having relatively short and relatively long filaments secured thereto in the manner of a pile, the short filaments carrying a substance which as compared with the silverware is preferentially susceptible to chemical attack by the tarnishing agents in the atmosphere, the long filaments being substantially free of such substance and projecting beyond the short and substantially hiding the same.

4. Material for protecting from tarnish silverware placed in adjacency thereto, comprising a backing having one face completely covered by a deep pile of textile fiber material the deep pile concealing a shorter pile of textile fiber material also anchored to said backing, the fibers of the short pile retaining therein a substance which as compared with the silverware is preferentially subject to chemical attack by tarnishing agents in the air, the long pile being substantially free of such substance.

ROBERT H. PREW.

REFERENCES CITED:

The following references are of record in the file of this patent:

UNITED STATES PATENTS

| Number    | Name           | Date           |
|-----------|----------------|----------------|
| 223,814   | Pennington     | Jan. 27, 1880  |
| 2,003,333 | Barnard et al. | June 4, 1935   |
| 2,014,426 | Dorogi         | Sept. 17, 1935 |
| 2,136,483 | Barnard        | Nov. 15, 1938  |
| 2,368,706 | Fountain       | Feb. 6, 1945   |
| 2,383,598 | Gliden         | Aug. 28, 1945  |
| 2,428,591 | Slayter        | Oct. 7, 1947   |